

# United States Patent [19]

Morris

[11] 4,448,839

[45] \* May 15, 1984

[54] **METHOD OF SIZING HYDROPHOBIC YARN**

[75] Inventor: **Hal C. Morris**, Warminster, Pa.

[73] Assignee: **Rohm and Haas Company**, Philadelphia, Pa.

[\*] Notice: The portion of the term of this patent subsequent to Jul. 19, 2000 has been disclaimed.

[21] Appl. No.: **312,761**

[22] Filed: **Oct. 20, 1981**

### Related U.S. Application Data

[63] Continuation-in-part of Ser. No. 311,561, Oct. 16, 1981, abandoned, and Ser. No. 202,543, Oct. 31, 1980.

[51] Int. Cl.<sup>3</sup> ..... **B32B 7/00; B65B 33/00; B05D 3/02**

[52] U.S. Cl. ..... **428/267; 8/115.6; 252/8.6; 427/155; 427/389.9; 427/393.4; 427/401; 428/245; 428/265**

[58] Field of Search ..... **427/389.9, 393.4, 155, 427/401; 428/245, 265, 394, 224, 267; 8/138, 115.6; 28/166; 252/8.6, 8.9**

[56]

### References Cited

#### U.S. PATENT DOCUMENTS

|           |         |                     |             |
|-----------|---------|---------------------|-------------|
| 2,807,865 | 10/1957 | Shippee .....       | 28/76 X     |
| 3,676,207 | 7/1972  | Lofton et al. ..... | 28/167 X    |
| 4,015,317 | 4/1977  | Johnsen .....       | 28/72.6     |
| 4,033,922 | 7/1977  | Baron et al. .....  | 28/76 X     |
| 4,106,900 | 8/1978  | Perkins .....       | 28/168 X    |
| 4,239,671 | 12/1980 | Fink et al. .....   | 28/76 X     |
| 4,248,755 | 2/1981  | Williams .....      | 28/167 X    |
| 4,312,914 | 1/1982  | Guth .....          | 427/393.4 X |

Primary Examiner—Thurman K. Page

Attorney, Agent, or Firm—Michael B. Fein; Harold L. Greenwald; George W. F. Simmons

[57]

### ABSTRACT

A method of sizing a hydrophobic yarn for weaving comprising the steps of applying thereto an acid pH latex of a free radical initiated vinyl polymer and drying the yarn. The polymer has a weight average molecular weight of from about 300,000 to about 2,500,000, and in dried film form is hydrophobic, not redispersible in a solution at a low pH and redispersible in an alkaline aqueous medium. The polymer is prepared from monomers comprising about 8% to about 14%, by weight ethylenically unsaturated acid. The average solubility parameter of the monomers in the polymer is between about 9.0 and about 9.5; the calculated polymer  $T_g$  is between about  $-20^{\circ}\text{C}$ . and  $20^{\circ}\text{C}$ . Preferred yarns are nylon and polyester.

13 Claims, No Drawings

**METHOD OF SIZING HYDROPHOBIC YARN**

This application is a continuation-in-part of application Ser. No. 311,561 filed Oct. 16, 1981, now abandoned, and of Ser. No. 202,543 filed Oct. 31, 1980.

**BACKGROUND OF THE INVENTION**

This invention relates to the sizing or dressing of yarns whether of spun or continuous filament type, to render them amenable to textile operations, for example, twisting, doubling, weaving, knitting, braiding and so forth. It is particularly concerned with sizes of the removable type which are adapted to be applied to hydrophobic yarns, such as polyester or nylon yarns, and especially yarns for use in water jet looms.

Various water-soluble or highly water dispersible polymeric colloidal substances, such as starch, polyvinyl alcohol and acid rich acrylic copolymers have been used for the sizing of yarns including moderately hydrophobic yarns such as nylon yarn, but such materials generally show insufficient adhesion to the more hydrophobic yarns such as polyester. This lack of adhesion requires the application of excessive amounts of sizing material to protect the filaments or fibers or to compensate for the tendency for the size to rub off on guides and other surfaces of the textile fabricating machinery. A suitable polymeric size must not be so hard or brittle as to shed particles during passage through the textile fabricating machinery nor may it adhere to the metal in preference to the fiber or yarn and in this way lead to deposits of size materials being left on metal drives or drying drums during the processing. Sizing of yarns for use in water jet looms presents particular problems because the shed opening on the looms is very small and electronic controls may be so fine that fuzzy yarns either transfer with the jets or tend to trip the stop motion in electronically controlled units which then stop the loom abruptly.

The acrylic copolymer size of the instant invention has excellent adhesion to a wide range of hydrophobic yarns and does not require extremely stringent drying conditions in order to develop good water resistance. Despite being highly hydrophobic, the polymer is readily removable with a mild alkali scour and thus is an excellent warp size for yarns to be woven on a conventional shuttled or shuttleless loom or preferably on a water jet loom. Additionally, the polymer is tack-free in film form and, being a latex emulsion as prepared, is readily amenable to dilution and dries easily under moderate conditions to a water-resistant tack-free polymer.

**BRIEF DESCRIPTION OF THE INVENTION**

This invention is a method of sizing hydrophobic yarns for weaving. The method comprises the steps of applying a certain latex to the yarn and drying the treated yarn. The latex has an acid pH and is a latex of a free radical initiated vinyl polymer having a weight average molecular weight between about 300,000 and 60 about 2,500,000. Said polymer, in dried film form, is hydrophobic and is not redispersible in an aqueous solution at a low pH, such as from about 2 to about 5 or preferably even to 7, and is redispersible in an alkaline aqueous medium. The polymer is a polymer of monomers having a volume average solubility parameter (S.P.) between about 9.0 and about 9.5; the monomers comprising about 8% to about 14%  $\alpha$ - $\beta$ -ethylenically

unsaturated acid. The glass transition temperature (Tg) of the polymer is between about -20° C. and 20° C.

**DETAILED DESCRIPTION**

The polymer latex of the instant invention is made, preferably by a gradual addition thermal process, at about 30% to 60% solids following conventional emulsion polymerization procedures such as taught in the books entitled *Emulsion Polymerization* by D. C. Blackley (Wiley, 1975) and by S. A. Bovey et al (Interscience Publishers, 1965) and *Applications of Synthetic Resin Emulsions* by H. Warson (E. Benn, Ltd., 1972) and *Emulsion Polymerization of Acrylic Monomers* (Rohm and Haas Co. bulletin CM104A/cf) all herein incorporated by reference. The polymer is preferably a linear polymer free of crosslinks and branch points. In one desirable embodiment, the polymer is prepared from monomers consisting essentially of, by weight, 45-65% butyl acrylate, 28-45% styrene or methyl methacrylate or a mixture thereof, 8-14% acrylic acid or methacrylic acid or a mixture thereof; preferably the monomers consist essentially of 50-60% butyl acrylate, 28-40% styrene and 10-13% acrylic acid or methacrylic acid. The polymer has a weight average molecular weight of from about 300,000 to about 2,500,000 with 500,000 to about 2,000,000 being preferred and 600,000 to 1,500,000 being most preferred.

The polymer latex forms a film on a hydrophobic yarn, preferably a polyester such as polyethylene terephthalate or a nylon such as nylon 66, or nylon 6. The film has excellent adhesion and flexibility thus providing a hard, tough, protective film unaffected by the abrasive action of looms, particularly water jet looms, and by humidities up to 100%. The polymer is easily removed by scouring with dilute aqueous solutions of alkaline materials.

The hydrophobic yarn of this invention comprises fibers which exhibit moderate to little uptake of water upon immersion in water or exposure to high humidity. This property is often measured by adsorption of water by a polymer film having a composition corresponding to that of the fiber or by the moisture regain or uptake of dehydrated fibers when held in an atmosphere of fixed relative humidity. Sources of such data are J. R. Scott and W. J. Roff, et al., *Handbook of Common Polymers*, CRC Press, Cleveland, Ohio, 1971; E. Sutermeister, *Chemistry of Pulp and Paper Making*, John Wiley & Sons, New York, 1941; and the periodical *Textile World*, McGraw-Hill Publications, Atlanta, Georgia. The following table is abstracted from the 1978 *Textile World* Man-Made Fibers Chart, herein included by reference on page 51 et seq. of the August 1978 *Textile World*.

| Fiber                      | Moisture Regain<br>(%/70° F./65% RH) |
|----------------------------|--------------------------------------|
| Polyethylene Terephthalate | 0.4                                  |
| Nylon 6                    | 2.8-5.0                              |
| Nylon 66                   | 4.0-4.5                              |
| Viscose Rayon              | 11-13                                |
| Cellulose Acetate          | 2.5-6.5                              |
| Acrylic (AN)               | 1.0-2.5                              |
| Modacrylic                 | 2.5-3.0                              |
| Polyethylene               | negligible                           |
| Polypropylene              | 0.01-0.1                             |
| Aramid                     | 4-7                                  |
| Kelvar ®, Nomex ®-DuPont   | 0                                    |
| Teflon ® (DuPont)          | ca. 1                                |
| Spandex (polyurethane)     |                                      |

-continued

| Fiber | Moisture Regain<br>(%/70° F./65% RH) |
|-------|--------------------------------------|
| Glass | none                                 |

Hydrophobic fibers are fibers wherein the moisture regain is about 5% or less, preferably between about 4.5%, and about 0.1% and most preferably between about 3% and 0.2% of the fiber weight at 70° F. and 65% R. H. The yarn of the present invention preferably comprises at least about 50% by weight of such hydrophobic fibers; more preferably the yarn consists essentially of hydrophobic fibers and most preferably entirely of hydrophobic fibers, especially 100% polyester fibers, such as poly (ethylene terephthalate), and 100% nylon fibers.

The amount of copolymer applied to the textile material may vary from about 1 to about 20% by weight of yarn depending on the purpose for which the application is intended and on whether or not auxiliary conditioning or sizing agents are included in the composition when it is applied to the textile. The latex may be applied by spraying, dipping, padding, by sizing rolls, transfer rolls or the like. An entire warp may be passed through a conventional slasher or a yarn may be individually treated in a single end sizer. The latex may have a concentration of 1-25% by weight solids in the aqueous system and excess may be removed, such as by squeeze rolls or wipers, and the treated yarn may then be dried. Drying may be effected by any suitable means such as by heated air or drying cans. Drying may be effected at a wide range of temperatures such as 70-120°C. The aqueous latex may be applied at room temperature or at elevated temperatures such as up to about 80°C. For warp sizing of spun yarns the preferred proportion of polymer applied to the yarn is from 5-15% by weight of the initial weight of the yarn. For the sizing of continuous filament yarns, including water jet loom sizing, the preferred proportion is from about 1% to about 10% copolymer on the weight of the yarn. The higher amount of size is needed for fine (low) denier zero or low twist yarn.

The copolymer of this invention may be applied to yarns to modify their properties and especially to render them more amenable to textile processing operation. Although not necessary, auxiliary materials may be incorporated into the latex such as surfactants or water dispersible lubricants, including sulfonated oils, self-dispersible waxes, swelling or plasticizing agents for the yarn, etc.

The article obtained, after application of the sizing composition to the yarn and drying, is essentially free from the disadvantage of developing static charges and loss of sizing material by transfer to guides or by shedding. Surprisingly, the sizing material is readily removed by common scouring operations because of the ready solubility in aqueous alkaline medium despite its marked hydrophobicity, affinity for hydrophobic fibers and insolubility in acid medium. Even mildly alkaline scour solutions, such as 0.15% soda ash, are completely effective in removal of this polymer. Such mildly alkaline solutions may have a pH about 11.

Various tests are employed to gauge the suitability of the polymer latex for use in sizing polyester yarn. The test methods are described below; in the examples there are data comparing polymers of the instant invention with materials of the prior art and with examples of

polymer latices outside the bounds of the instant invention.

The adhesion of the polymer to the yarn as measured by the Sand Tumble Test, described below, gauges how well a yarn bundle will resist abrasion on the loom. Run under dry conditions the test relates to performance on a standard loom and run under wet conditions the test relates to performance on a water jet loom. A value of 50 is considered acceptable although 75 is preferred and values about 100 are most preferred.

The Adhesion to Mylar® Test is indicative of adhesion, especially to a polyester substrate since Mylar is a polyester substrate. The Crinkle Test gives the tendency of the polymer to flake from the substrate under flexing, thus simulating a yarn going over a roller or a guide. Flaking under such conditions would cause a weak spot in the yarn and thus lead to breaks in the yarn on the loom. The Scrape Test is to simulate the action at drop wires or a reed in the loom and also gives a gauge of the film toughness which property is required for runability in a mill.

Water Resistance Tests measure a property needed for good performance in a water jet loom. Low water resistance is indicative of high swelling which leads to a markedly weaker film and thus to a weak sized yarn. The Moisture Regain measure, being at 95% relative humidity, additionally indicates the stability of the sized yarn to changes in ambient conditions such as seasonal or from dry day to humid day.

Tack Test measures the ability of the sized and dried yarn to be rolled on a beam while warm and then be unrolled from the beam without sticking.

Removability of the size is, of course, essential with the final test of removability from the sized yarn being most important. The size should be completely removable from the yarn.

The polymer of the instant invention is applied to the yarn in the form of a latex of particles usually about 0.07 to about 0.25 microns diameter, with 0.10 to 0.18 being preferred and about 0.14, or a range within about 0.02 of that value, being most preferred. Polymerization procedures useful in producing polymers of the desired particle size and molecular weight are given in the books referred to above. This highly hydrophobic polymer composition is applied at acid pH and is scoured at basic pH thus the polymer is intrinsically stronger, as a size, than a solution polymer would be in this application. The solution polymer would have to be at least partially neutralized to be in aqueous solution and thus would be highly swollen and weaker than the very hydrophobic latex polymer at low pH, of the instant invention. If attempts are made to have the solution polymer be more hydrophobic, and thus marginally soluble, then the difficulty of scouring increases. A further advantage of utilizing a latex versus an alkaline solution or dispersion of a polymer is that less severe drying conditions are required for the latex, a particularly significant energy saving.

Alternative embodiments of the instant invention may employ other ethylenically unsaturated monomers in the preparation of the polymer latex. In alternative embodiments it is preferred that the acid content and identity be the same as in the above-described embodiments although other  $\alpha$ - $\beta$  ethylenically unsaturated acids, such as itaconic acid, may be used. The acid level remains at 8% to 14% with 10% to 13% being preferred. Replacements for the butyl acrylate, styrene and methyl methacrylate are made on the basis that the

range of glass transition temperatures, ( $T_g$ ), calculated for a high molecular weight polymer, and S. P. are to remain within the range implicit in the compositional range for the embodiments taught above. Likewise preferred and more preferred are ranges of  $T_g$  and S. P. corresponding to the preferred and more preferred compositional ranges recited above.

Polymer Handbook, 2nd Edition, J. Brandrup and E. H. Immergut, editors (John Wiley & Sons, New York, 1975) section IV, part 15, entitled "Solubility Parameter Values" by H. Burrell, on pages IV-337 to IV-359, herein incorporated by reference, defines S. P., describes how it is determined or calculated, contains tables of S. P. and gives further references to scientific literature on S. P. Table I on pages IV-341 to 344 lists the S. P. of solvents, including many monomers thereunder. In this specification numerical values of S. P. have the dimensions (calories per cubic centimeter) to the one half power, i.e. (cal./cc.)<sup>0.5</sup>. The S. P. is the square root of the cohesive energy density which in turn is the numerical value of the potential energy of 1 cc of material, the potential resulting from the Van der Waals attraction forces between the molecules of a liquid or solid. Burrell describes a number of ways of calculating S. P. from experimentally determined physical constants and two ways of calculating them from the structural formula of a molecule. The structural formula methods are normally used when the data for the calculation from physical constants are not available or are considered particularly unreliable. Calculation from the structural formula utilizes tables of group molar attraction constants such as those given on pages IV-339. The table of Small is preferred. The S. P. concept may be considered an extension of the old rule "Like dissolves like." recognized since the early days of chemistry.

As tables of the solubility parameter of monomers are available, as noted above, it is convenient to define a polymer in terms of the solubility parameter of the monomers employed in its polymerization. The effective solubility parameter of a mixture is the sum, over the (i) components of the mixture, of the product of the volume fraction of the component (vi) times its S. P., i.e., S. P. (mixture) =  $\sum V_i (S. P.)$ ; according to Scott and Magatt (See

Encyclopedia of Polymer Science and Technology, Vol. 3, John Wiley, 1965, page 856). The volume fraction of each component is calculated from the weight fraction and the known density of the component of the monomer mixture assuming no changes in volume on mixing. Densities of the monomers are available in the usual sources such as *The Polymer Handbook*, *The Encyclopedia of Polymer Science and Technology*, and the manufacturers of the various monomers. The range of S. P. of the monomers employed in the polymers of the instant invention is from about 9.0 to 9.5 with the range 9.1 to 9.4 being preferred.

The calculated  $T_g$  of a polymer is determined by the equation of T. G. Fox, Bull. Am. Physics Soc. 1,3, page 123 (1956) based on the  $T_g$  of homopolymers of the individual monomers in the copolymer. Tables of the  $T_g$  of homopolymers are given in "Polymer Handbook," section III, part 2, by W. A. Lee and R. A. Rutherford herein incorporated by reference.  $T_g$  values referred to herein are calculated  $T_g$  values for high molecular weight polymers. The polymers of this invention have a  $T_g$  from about -20° C. to about 20° C. with the range -10° C. to +10° C. being preferred.

Other monomers which can be used in these alternative embodiments are preferably vinyl aromatic hydro-

carbons, such as vinyl toluene and alpha methyl styrene; alkyl acrylates wherein the alkyl group has 1 to 8 carbon atoms, such as ethyl acrylate, propyl acrylate, and 2-ethylhexyl acrylate; alkyl methacrylates having 2 to 4 carbon atoms, such as ethyl methacrylate and isobutyl methacrylate and acrylonitrile.

The vinyl polymer used in the present invention is made as an aqueous dispersion of an emulsion polymer at about 40% to 60% by weight of polymer solids.

10 Monomers can be selected from the group consisting of C<sub>2</sub>-C<sub>18</sub> alkyl acrylates, C<sub>2</sub>-C<sub>18</sub> alkyl methacrylates, vinyl aromatic compounds, vinyl halides, vinylidene halides, vinyl esters of saturated carboxylic acids, other polymerizable ethylenically unsaturated monocarboxylic and dicarboxylic acids and esters thereof, acrylonitrile, methacrylonitrile and alpha-olefins. Examples of the C<sub>2</sub>-C<sub>18</sub> alkyl groups of the esters of acrylic and methacrylic acids which are useful in forming the polymers of this invention include methyl, ethyl, n-butyl, i-butyl, sec-butyl, t-butyl the various isomeric pentyl, hexyl, heptyl, and octyl (especially 2-ethylhexyl), isobornyl, decyl, lauryl, cetyl, stearyl and like groups. Examples of useful vinyl aromatic compounds include styrene and derivatives thereof such as vinyl toluene and alpha-methyl styrene; of vinyl and vinylidene halides are the corresponding chloride compounds; of vinyl esters of saturated carboxylic acids include vinyl acetate and vinyl propionate; of polymerizable ethylenically unsaturated monocarboxylic and dicarboxylic acids include acrylic acid, methacrylic acid, itaconic acid and crotonic acid; and of alpha-olefins include ethylene, propylene, and butylene.

In the following examples parts and percentages are by weight and temperature in degrees Celsius unless otherwise indicated. The examples illustrate the invention and are not to be construed as limiting the invention thereto. As given below, a general method was followed in the preparation of yarns and films. The method was followed throughout the examples unless an exception is noted in a given example. The same is true of the general test methods given below.

#### Preparation of Materials

45 **Sized Yarns:** The latex, at a pH of ca. 2.0 to 2.5 as prepared, or at a higher acid pH such as about 4 or 5, is diluted to 8% resin solids with water and applied to polyester or nylon filament yarn at room temperature on a laboratory size single end slasher. The slasher employs a double squeeze and consists of an immersion bath followed by a metal drum and two Teflon ®-coated drums, the first squeeze being between the metal drum and the first Teflon coated drum and the second squeeze between the two Teflon coated drums. The slasher is run at 4M/min and the sized yarn is dried 15 seconds thru a tube dryer set at 115° C. All sized yarn is conditioned one day at 21° C. and 60% R. H. before testing.

50 **Film Preparation:** 20 mil films are prepared by diluting the latex with water to the necessary solids content per volume. The diluted latex is then poured into a polypropylene culture dish, placed in a dust free area on a level surface, and air dried for 4 days or until a clear film is obtained. Thinner films (about 0.2 mils) are prepared by pouring a 15% solids latex, obtained by dilution with warm water (54° C.), onto a two mil Mylar ® sheet. The films are room dried overnight, then oven dried for one minute at 110° C.

## Test Methods

Adhesion by Sand Tumble Test: The sized yarns are evaluated for wet and dry adhesion using laboratory sand tumble tests. Dry — Duplicate 3 yd. skeins of the sized yarn are placed in an 8 oz. jar containing 150g of coarse sand, rotated for 30 minutes on an Atlas Launder-ometer®, removed and rated for % of the fiber bundle remaining intact. Wet — The same procedure is followed except the jar now contains 50g of sand and 150g water. Ratings are made the same way.

Adhesion to Mylar: The adhesion of the thin film is determined by two methods, scrape and crinkle. The scrape test consists of scraping the film with a razor blade and counting the number of strokes required to remove the polymer film from the polyester sheet. The crinkle test is designed to measure the film adhesion to polyester sheet by crumpling the sheet by hand and flattening it, noting any film separation from the Mylar. In the scrape test the results are classed as follows: Poor 1-2, Fair 3-4, Good 5 and Excellent 6 or more strokes. Crinkle test results are judged: Excellent—no change of Fair—cracks and slight film removal.

Water Resistance: The wet sand tumble test, previously noted, is a preliminary screen test of the water resistance. All additional testing of this property is conducted on the polymer films, either free or on Mylar, as follows: One inch squares of both the free and Mylar films are placed in 30° C. water for 30 minutes and evaluated for any change in clarity, toughness, adhesion, and size using the following ratings: Excellent=no change; Good=film swelling and Fair=swelling and loss of toughness. The 20 mil free film is also evaluated for moisture regain when first bone dried and then subjected to 95% RH in a constant humidity chamber; the film is also observed for degree of haze developed.

Tack: The tackiness of the polymer is evaluated, immediately following one minute drying at 110° C., on the film cast on Mylar. For this evaluation, two films on Mylar are pressed film/film and then opened to gauge adhesion.

Removeability of the Size: This property is evaluated by two methods, alkali solubility of the film, and an actual scouring of sized yarn. Solubility of the film is

determined by placing of a  $\frac{1}{4}$ " square of the 20 mil free film in a 1%  $\text{Na}_2\text{CO}_3$  solution at 70° C. and recording the time it takes to dissolve up to 20 min. at which time the level of incomplete solution is gauged. The sized yarn is evaluated for size removal by scouring the yarn at 70-74° C. for 30 minutes in a 1.0%  $\text{Na}_2\text{CO}_3$  and 0.1% surfactant (Triton®-X-100) bath with mild agitation. The yarns are rinsed five minutes in warm water (54° C.) and then cold water. The degree of removeability is determined by dyeing scoured and control yarns in Basic Red #14 at 60° C. and observing the dye pickup.

The following abbreviations are used in the examples below: BA butyl acrylate, St styrene, AA acrylic acid, MMA methyl methacrylate, MAA methacrylic acid, EA ethyl acrylate, EGDMA ethyleneglycol dimethacrylate,  $\beta$ BMA isobutyl methacrylate, VT vinyl toluene, MeST  $\alpha$ -methyl styrene, AN acrylonitrile, 2-EHA 2-ethylhexyl acrylate, PMA propyl methacrylate, and EMA ethyl methacrylate.

## EXAMPLE 1

## Copolymers Containing 12% Acrylic Acid

Film and yarn are prepared using acrylic copolymer latex samples described in Table I below. The yarn being sized is Milliken textured polyester yarn, Saluda 373, 70 Denier, 33 filament, 1 twist. The test results, in Table I below, show that the samples varying in butyl acrylate content from 45% to 50.5% are all suitable sizing polymers compared to two commercial materials (1D, 1E). All of the examples exhibited no tack, except 1D which had slight tack when hot. The viscosity average molecular weight of the polymer of Example 1A is about 1.2 to 1.3 million.

## EXAMPLE 2

## Copolymers of 12% Methacrylic Acid

Using the same yarn as in Example 1 methacrylic acid containing polymers having 55-60% butyl acrylate are tested with the results found in Table II. An additional observation made is that the methacrylic acid samples produced less foam in the bath and during handling than the corresponding acrylic acid samples. All of the examples exhibited no tack. The weight average molecular weight of the polymer in Example 2C is about 600,000 to 700,000.

TABLE I

| Ex.             | Composition                           | $T_g$<br>°C. | S. P. <sup>5</sup> | Sand<br>Tumble |         | Film<br>Solubility<br>(min.) | Removability<br>from<br>yarn | Water<br>Resistance<br>of films |              | Adhesion to<br>Mylar |         | Moisture<br>Regain<br>(%) |
|-----------------|---------------------------------------|--------------|--------------------|----------------|---------|------------------------------|------------------------------|---------------------------------|--------------|----------------------|---------|---------------------------|
|                 |                                       |              |                    | Dry            | Wet     |                              |                              | 20 mil                          | Mylar        | Scrape               | Crinkle |                           |
| 1A <sup>2</sup> | 50.5 BA/37.5<br>St/12 AA              | 3            | 9.4                | 100            | ca. 100 | Partial <sup>1</sup>         | Complete                     | Exc.                            | No<br>Change | Exc.                 | Exc.    | 3.0                       |
| 1B <sup>2</sup> | 50.5 BA/37.5<br>St/12 AA              | 3            | 9.4                | 75-100         | 75      | Partial                      | Complete                     | Good                            | No<br>Change | Exc.                 | Exc.    | 3.7                       |
| 1C              | 45 BA/43 MMA/<br>12 AA                | 12           | 9.2                | 75-100         | 75      | <19                          | Complete                     | Good-<br>Exc.                   | No<br>Change | Exc.                 | Exc.    | 3.5                       |
| 1D              | Polyester <sup>3</sup><br>Eastman MPS |              |                    | 50             | 25      | <4                           | Complete                     | Good                            | No<br>Change | Exc.                 | Exc.    | 22.0                      |
| 1E              | Acrylic <sup>4</sup><br>ABCO FT-2B    |              |                    | ca. 100        | 75      | <20                          | Complete                     | Exc.                            | No<br>Change | Poor                 | Good    | 11.0                      |

<sup>1</sup>Partial - some film remaining after 20 minutes.<sup>2</sup>Latex particle diameter is 0.10 micron in Example 1A and 0.21 in Example 1B.<sup>3</sup>Applied as an 8% solids solution at a pH of 6.<sup>4</sup>Applied as an 8% solids solution at a pH of 8.<sup>5</sup>In (calories per cubic centimeter) 0.5

TABLE II

| Ex.             | Composition           | T <sub>g</sub><br>°C. | S. P. | Sand<br>Tumble |         | Film<br>Solubility<br>(min.) | Removability<br>from<br>yarn | Water<br>Resistance<br>of films |              | Adhesion to<br>Mylar |         | Moisture<br>Regain<br>(%) |
|-----------------|-----------------------|-----------------------|-------|----------------|---------|------------------------------|------------------------------|---------------------------------|--------------|----------------------|---------|---------------------------|
|                 |                       |                       |       | Dry            | Wet     |                              |                              | 20 mil                          | Mylar        | Scrape               | Crinkle |                           |
| 2A <sup>1</sup> | 57 BA/31<br>St/12 MAA | -1                    | 9.2   | 75             | 75      | Partial                      | Complete                     | Exc.                            | No<br>Change | Good-<br>Exc.        | Exc.    | 2.0                       |
| 2B              | 60 BA/28<br>St/12 MAA | -5                    | 9.2   | 50-75          | 50-75   | Partial                      | Complete                     | Exc.                            | No<br>Change | Exc.                 | Exc.    | 2.0                       |
| 2C <sup>1</sup> | 57 BA/31<br>St/12 MAA | -1                    | 9.2   | ca. 100        | ca. 100 | Partial                      | Complete                     | Exc.                            | No<br>Change | Exc.                 | Exc.    | 2.1                       |
| 2D              | 55 BA/33<br>St/12 MAA | 2                     | 9.2   | 75-100         | 75      | Partial                      | Complete                     | Exc.                            | No<br>Change | Good-<br>Exc.        | Fair    | 1.8                       |

<sup>1</sup>Latex particle diameter is 0.08 micron in Example 2A and 0.13 micron in Example 2C.

## EXAMPLE 3

## Compositional Variations

Polymer latexes of various compositions, as reported in Table III below, are used to prepare films and size 20 yarns as in Example 1. The results in Table III indicate that the polymer based on ethyl acrylate (3C) has low adhesion, both by the sand tumble test and the two

## EXAMPLE 4

## Utilization of Other Monomers

Using the same yarn as in Example 1 other polymers are tested resulting in the data in Table IV. All of the examples are suitable for use in the water jet loom although Example 4A appears to be somewhat less so than the others.

TABLE IV

| Ex-<br>am-<br>ple | Composition               | T <sub>g</sub> | S. P. | Sand<br>Tumble <sup>1</sup> |        | Film<br>Solu-<br>bility<br>(min.) | Removability<br>From<br>Yarn | Water<br>Resistance<br>of Films |              | Adhesion to<br>Mylar |               | Moisture <sup>2</sup><br>Regain<br>(%) |
|-------------------|---------------------------|----------------|-------|-----------------------------|--------|-----------------------------------|------------------------------|---------------------------------|--------------|----------------------|---------------|----------------------------------------|
|                   |                           |                |       | Dry                         | Wet    |                                   |                              | 20 mil                          | Mylar        | Scrape               | Crinkle       |                                        |
| 4A                | 45 BA/45 i-BMA/<br>10 MAA | 3° C.          | 9.35  | 75                          | 75     | Partial                           | Complete                     | Good                            | Sl.<br>Haze  | Good-<br>Exc.        | Exc.          | 4.3                                    |
| 4B                | 57 BA/31 VT<br>12 MAA     | -1° C.         | 9.26  | 75-100                      | 75-100 | Partial                           | Complete                     | Exc.                            | No<br>Change | Exc.                 | Good-<br>Exc. | 4.1                                    |
| 4C                | 58 BA/28 MeSt/<br>14 AA   | 1° C.          | 9.16  | 75-100+                     | 75-100 | Partial                           | Complete                     | Exc.                            | No<br>Change | Exc.                 | Good-<br>Exc. | 7.8                                    |
| 4D <sup>1</sup>   | 57 BA/31 St/<br>12 MAA    |                |       | 75-100                      | 75-100 | Partial                           | Complete                     | Exc.                            | No<br>Change | Exc.                 | Good-<br>Exc. | 3.5                                    |

<sup>1</sup>Example 4D is a repeat preparation of the latex of Example 2C

<sup>2</sup>Humidity during this test was 100% R. H. therefore results are slightly higher than normal 95% R. H. test.

adhesion to Mylar tests, is high in moisture regain and produces a hazy film when tested for water resistance of 40 a thin film on Mylar. Example 3D, having 4% acid in the copolymer, exhibits an insoluble film and less than complete removability from the yarn upon scouring and slightly hazy thin film on Mylar in the water resistance test. Example 3E, having 16% acid in the copolymer, 45 also shows less than complete removability from the yarn on scouring and in addition has limited water resistance shown by both the 20 mil film and the thin film results. The only examples, in this group, exhibiting tack are 3C which has some tack when hot and 3D which has some tack even when cooled to room temperature.

40

50

## EXAMPLE 5

## Nylon Yarn

The procedure of Example 1 is followed with nylon 45 yarn being substituted for the polyester yarn of Example 1. The nylon yarn employed is DuPont 70 denier, 34 filament, 0 twist yarn. The test results, in Table V below, show that the polymer of Example 4D compares favorably with materials commercially available. The nylon employed is identified as 70-34-R25 295 M. D. pirn 13073.

TABLE III

| Ex. | Composition                            | T <sub>g</sub><br>°C. | S. P. | Sand<br>Tumble |         | Film<br>Solubility<br>(min.) | Removability<br>From<br>Yarn | Water<br>Resistance<br>of Films |              | Adhesion to<br>Mylar |         | Moisture<br>Regain<br>(%) |
|-----|----------------------------------------|-----------------------|-------|----------------|---------|------------------------------|------------------------------|---------------------------------|--------------|----------------------|---------|---------------------------|
|     |                                        |                       |       | Dry            | Wet     |                              |                              | 20 mil                          | Mylar        | Scrape               | Crinkle |                           |
| 3A  | 50.5 BA/37.5<br>MMA/12 AA              | 4                     | 9.2   | 75             | 75      | <15                          | Complete                     | Good-<br>Exc.                   | No<br>Change | Good                 | Exc.    | 5.0                       |
| 3B  | 48.5 BA/37.5<br>St/14 AA               | 5                     | 9.4   | 100            | ca. 100 | Partial                      | Complete                     | Exc.                            | No<br>Change | Fair-<br>Good        | Good    | 4.0                       |
| 3C  | 65 EA/22.8<br>MMA/12 MAA/<br>0.2 EGDMA | 16                    | 8.9   | 50             | 50      | <4                           | Complete                     | Good                            | Hazy         | Poor                 | Fair    | 11                        |
| 3D  | 58.5 BA/37.5<br>St/4 AA                | -9                    | 9.1   | 75             | 75+     | Insol.                       | Almost<br>Complete           | Exc.                            | Sl.<br>Hazy  | Exc.                 | Exc.    | 4                         |
| 3E  | 46.5 BA/37.5<br>St/16 AA               | 8                     | 9.5   | 100            | 100     | Partial                      | Almost<br>Complete           | Fair-<br>Good                   | Hazy         | Good-<br>Exc.        | Exc.    | 6                         |

The latex of Example 3C is neutralized with ammonia to a pH of 7.5 and utilized as a solution.

EXAMPLE 6  
Other Compositions

Polymer latexes of a number of different compositions applied to the yarn of Example 1 and films prepared from the latex have wet and dried adhesion which are acceptable as is the adhesion to Mylar by scrape and crinkle, the water-resistance of the film, the moisture regain, tack, solubility of the film, and removability of the polymer from the yarn. Polymer compositions, calculated  $T_g$  values and solubility parameter values are given in Table VI.

TABLE V

|                                | Example 4D             | Dow XD-8959.00                     | ABCO BY-4                   |
|--------------------------------|------------------------|------------------------------------|-----------------------------|
| <u>Physical Properties</u>     |                        |                                    |                             |
| Appearance                     | Milky white, fluid     | White, fluid                       | Yellow, fluid               |
| Solids                         | 29%                    | 25%                                | 21%                         |
| pH                             | 2.3                    | 9.2                                | 6.3                         |
| Film (20 mil)                  | Firm, slightly brittle | Clear, pieces <sup>1</sup>         | Yellow, hard and brittle    |
| Composition                    | BA/St/MAA              | Ethylene/Acrylic Acid <sup>2</sup> | BA/MMA/AN/acid <sup>2</sup> |
| $T_g$ (measured)               | 12° C.                 | 35° C.                             | 36° C.                      |
| <u>Performance</u>             |                        |                                    |                             |
| Sand Tumble <sup>3</sup> , Dry | 100                    | 100                                | 75                          |
| Wet                            | 75-100                 | 75-100                             | 50                          |
| Removability, Yarn             | Partial                | Partial                            | Partial                     |
| Film Solubility                | under 35 min.          | over 38 min.                       | under 14 min.               |
| Water Resistance (20 mil)      | Excellent              | Excellent                          | Very Poor                   |
| Moisture Regain                | 4.0%                   | 2.0%                               | 24%                         |

<sup>1</sup> Does not form a continuous film on drying at room temperature.

<sup>2</sup> Acid content determined by neutralization is XD-8959.00 - 12%, BY-4 - 23%; unidentified minor components may be present.

<sup>3</sup> Nylon yarn sized using same conditions as polyester yarn - 8% solution.

TABLE VI

| EXAM-<br>PLE | COMPOSITION                | $T_g$ | SOLUBILITY<br>PARAMETER |
|--------------|----------------------------|-------|-------------------------|
| 6A           | 45 BA/42 iBMA/13 AA        | -2    | 9.39                    |
| 6B           | 57 BA/33 iBMA/10 MAA       | -10   | 9.35                    |
| 6C           | 54 BA/32 MeST/14 AA        | 8     | 9.10                    |
| 6D           | 58 BA/28 MeST/14 AA        | 1     | 9.16                    |
| 6E           | 60 BA/28 MeST/12 MAA       | 4     | 9.13                    |
| 6F           | 46 BA/40 VT/14 AA          | 9     | 9.20                    |
| 6G           | 63 BA/28 VT/9 MAA          | -10   | 9.16                    |
| 6H           | 51 2-EHA/<br>41 MMA/8 AA   | 6     | 9.36                    |
| 6I           | 63 2-EHA/<br>28 MMA/9 MAA  | -6    | 9.13                    |
| 6J           | 50 2-EHA/42 St/8 AA        | 6     | 9.25                    |
| 6K           | 61 2-EHA/28 St/11 AA       | -8    | 9.11                    |
| 6L           | 53 2-EHA/<br>33 PMA/14 MAA | -5    | 9.11                    |
| 6M           | 41 2-EHA/<br>45 PMA/14 AA  | 0     | 9.18                    |
| 6N           | 60 2-EHA/<br>26 EMA/14 MAA | -7    | 9.11                    |
| 6P           | 65 2-EHA/<br>21 St/14 MAA  | -7    | 9.18                    |
| 6Q           | 45 2-EHA/<br>46 EMA/9 MAA  | 5     | 9.11                    |

I claim:

1. A method of sizing a hydrophobic yarn for weaving comprising the steps of (1) applying thereto an acid pH latex of a free radical initiated vinyl polymer having a weight average molecular weight of from about 300,000 to about 2,500,000; said polymer, in dried film

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9

UNITED STATES PATENT AND TRADEMARK OFFICE  
CERTIFICATE OF CORRECTION

PATENT NO. : 4,448,839

DATED : May 15, 1984

INVENTOR(S) : Hal C. Morris

It is certified that error appears in the above-identified patent and that said Letters Patent is hereby corrected as shown below:

In Claim 1, Column 12, line 5 after -20°C insert --to about 20°C--.

**Signed and Sealed this**

*Twenty-second Day of January 1985*

[SEAL]

*Attest:*

DONALD J. QUIGG

*Attesting Officer*

*Acting Commissioner of Patents and Trademarks*